

## UNITED STATES PATENT OFFICE.

WALTER BROADBRIDGE, EDWIN EDSER, AND WILLIAM WARWICK STENNING, OF LONDON, ENGLAND, ASSIGNEES TO MINERALS SEPARATION NORTH AMERICAN CORPORATION, OF NEW YORK, N. Y., A CORPORATION OF MARYLAND.

## PRODUCTION OF BRIQUETTES.

No Drawing.

Application filed August 17, 1920. Serial No. 404,106.

To all whom it may concern:

Be it known that we, WALTER BROADBRIDGE, EDWIN EDSER, and WILLIAM WARWICK STENNING, subjects of the King of England, all residing at London, England, have invented certain new and useful Improvements in the Production of Briquettes, of which the following is a specification.

This invention relates to the production of 10 briquettes, and particularly to the production of coal briquettes, and with coal concentrated from impure coal, coal dumps and the like.

One of the problems in briquetting is to 15 secure an efficient coating of the coal particles by the binding medium, such as pitch, tar, resin, and the like.

In the froth-flotation process of concentrating ores as disclosed in Patent No. 20 835120, to Sulman, Picard and Ballot, of November 6, 1906, and later patents, it is known that the methods therein used for agitating a pulp of ore and water with an 25 added agent, such as oil, tar and the like, result in a very effective coating of certain mineral particles with the added agent, and an equally effective flocculation of the particles which become readily separable from water, and we have now discovered by experiment that when finely divided coal in 30 suspension in water is subjected to similar types of agitation in the presence of a liquefied binding medium, the coal particles become readily and thoroughly coated and 35 also flocculated.

A feature of this invention, therefore, lies in the making of briquettes from carbonized fuel, whether artificially or naturally carbonized, as coal by a process wherein the 40 powdered coal, suspended in water, is subjected to agitation with a binding medium, whereby the coal particles are coated with the binding medium and flocculated so as to be readily separable from water.

Again, in the froth-flotation process of concentrating ores it was frequently found desirable to add to the aqueous pulp certain agents which facilitates the segregation of the desired mineral particles. In this specification such agents are referred to as 45 flocculating agents, and it may be desirable to

employ such an agent. Further, it is desirable that such agent, if employed, should itself subsequently assist as a binding agent in the briquetting. 55

A further feature of this invention, therefore, consists in the employment in the pulp, during the above described agitation, of a flocculating agent, such as slaked lime, which assists in the flocculation and subsequent 60 draining of the coated coal particles, and also acts as an auxiliary binding agent in briquetting.

Again, in the froth-flotation process of ore concentration, the action of the air in causing 65 flocculation and rendering the concentrate particles readily separable from water is known, and it is a feature of this invention that the agitation of the coal-water pulp with the binding agent is conducted with a greater 70 or less degree of aeration, either by agitation affecting or accompanied by the introduction of air or by air-agitation.

One process of producing coal briquettes from impure coal, coal dumps and the like, 75 according to this invention consists in crushing the crude material, if necessary, subjecting it to concentration by the froth-flotation process, agitating the concentrates in aqueous suspension with liquefied binding medium, 80 such as melted pitch, with or without tar, resin and the like, and with or without a flocculating agent, such as slaked lime, so that the concentrated coal particles become coated with the binding medium and flocculated, separating the resulting coal from 85 superfluous water and making the coal into briquettes.

## Example No. 1.

This test was carried out on flotation concentrates obtained by treating ground coal from a South Durham colliery, a bituminous, coking coal. The concentrates contained 15% of moisture, and 470 grammes 90 containing 400 grammes of dry coal were used. The concentrates were made into a 4:1 pulp with water; while the pulp was being vigorously agitated and aerated 28 grammes of melted pitch (7% of the dry 95 coal) were added. The pulp was then filtered and on examination it became evident 100

that the pitch was distributed over the coal particles, no separate particles of pitch being detectable. The filtered material was then heated, masticated, and kneaded, and finally 5 pressed in a die under 300 atmospheres pressure.

The resulting briquette was hard, homogeneous and free from cracks and fissures. It was superior in all respects to another briquette made from the same concentrates by 10 drying these, adding hard pitch that had been ground to pass 80 mesh, heating, masticating and kneading, finally pressing in a die under 300 atmospheres pressure.

15 In the process just described the coated coal is not floated after coating with the binding medium, but this may be done if desired by employing a suitable frothing agent and by conducting the agitation and 20 aeration in a suitable manner. Thus, the agent added may contain a small proportion (conveniently less than 1% on the coal) of coal tar oil or of cresol, either of which is a very effective frothing agent.

25 Thus, a modified method of producing coal briquettes according to this invention consists in crushing the crude material if necessary, subjecting it to concentration by the froth-flotation process, agitating the 30 concentrates in aqueous suspension with a liquid agent which affords or contains both a frothing agent and a binding medium, and with or without a flocculating agent, such as slaked lime, whereby the coal particles become coated with the binding medium, 35 flocculated and floated in the form of agglomerates supported by bubbles, collecting and draining the agglomerates and making the moist coal concentrates into 40 briquettes.

*Example No. 2.*

Similar coal concentrates were used as in Example No. 1. After the pitch had 45 been added to the wet pulp, cresol was added at the rate of 1 lb. to the ton of dry coal, and the pitch-coated coal was floated, removed, and filtered, a briquette being made by the method described above. 50 The briquette was equally as good as that obtained in the preceding test.

The concentration of the coal by the froth-flotation process, and the coating of the coal particles with the binding medium may 55 be combined into one single operation which may conveniently be a continuous operation.

Thus, another process of making coal briquettes from impure coal, coal dumps 60 and the like, according to this invention, consists in crushing the crude material, if necessary, subjecting it to concentration by flotation with the addition of a liquid agent which affords or contains both a frothing

agent and a binding medium, and with or 65 without a flocculating agent, such as slaked lime, whereby the coal particles become coated with the binding medium, flocculated and floated in the form of agglomerates supported by bubbles, while the gangue is not 70 so floated, collecting and draining the agglomerates and making the moist coal concentrate into briquettes.

*Example No. 3.*

75

In this test a slurry obtained from a bituminous coking coal, containing 17% of ash, was used, 400 grammes being made into a 4:1 pulp with water in a slide machine; 5% of melted pitch was added and cresol 80 at the rate of 1½ lbs. per ton of the crude slurry, and kerosene oil at the rate of 1½ lbs. per ton of the crude slurry. The pitch-coated coal was floated, removed, filtered, masticated, kneaded and briquetted, and a 85 briquette was made as described above. The briquette was of excellent qualities and contained 7½% of ash.

In cases where it is desired to recover the 90 coated coal as a float, it is preferred to employ an agitation apparatus of the subaeration type, such, for example, as are disclosed in the patents to Arthur Howard Higgins and one of us, William Warwick Stenning, 95 No. 1,155,815, to said Arthur Howard Higgins, No. 1,155,816, and to Thomas MacKellar Owen, No. 1,155,836, each dated October 5, 1915.

In any of the above described agitations, 100 the aqueous pulp may be heated to any desired degree to assist in disseminating the binding medium over the surface of the coal particles; and as the water is conveniently employed in closed circuit, its temperature can be kept up without much expense.

105 The result of all of the above described agitations with binding medium present is to form flocculations which are in fact agglomerations. The agglomerations tend to 110 free themselves from the water of the pulp and therefore a very low moisture content is readily attainable and is much more readily attainable than in the case of froth flotation concentrates from ore concentration.

115 The binding agents employed may be melted pitch, tar, resin and the like, or admixtures thereof. The flocculating agents may be slaked lime, sodium silicate and the like, referred to as saline flocculating agents.

120 What we claim as our invention and desire to secure by letters patent is:—

1. A process of making briquettes which 125 consists in suspending suitably divided solids in water so as to form a freely flowing pulp and subjecting the pulp to agitation with a binding medium having an affinity for solid particles so as to coat them with binding medium and agglomerate them, and

separating the resulting agglomerates from pulp liquid and forming the same into briquettes.

2. A process of making briquettes of carbonized fuel which consists in agitating the carbonized fuel in suitably divided condition in a freely flowing pulp with a binding medium having an affinity for carbonized particles so as to coat carbonized particles 5 with binding medium and agglomerate them, and separating the resulting agglomerates from pulp liquid and forming the same into briquettes.

3. A process of making briquettes which 15 consists in suspending suitably divided solids in water so as to form a freely flowing pulp, adding to the pulp a flocculating agent and also a binding medium, subjecting the pulp to agitation whereby solid particles 20 are coated with binding medium and flocculated so as to be readily separable from water, separating the coated particles from superfluous water, and forming them into briquettes.

25 4. A process of making briquettes which consists in suspending suitably divided solids in water so as to form a freely flowing pulp, adding to the pulp a saline flocculating agent and also a binding medium, subjecting the 30 pulp to agitation, whereby solid particles are coated with binding medium and flocculated so as to be readily separable from water, separating the coated particles from superfluous water, and forming them into briquettes.

35 5. A process of making briquettes from carbonized fuel which consists in suspending suitably divided carbonized fuel in water so as to form a freely flowing pulp, adding to the pulp a flocculating agent and also a binding medium, subjecting the pulp to agitation whereby carbonized particles are 40 coated with binding medium and flocculated so as to be readily separable from water, separating the coated particles from superfluous water, and forming them into briquettes.

45 6. A process of making briquettes from carbonized fuel which consists in suspending suitably divided carbonized fuel in water so as to form a freely flowing pulp, adding to the pulp a saline flocculating agent and also a binding medium, subjecting the pulp to agitation, whereby carbonized 50 particles are coated with the binding medium and flocculated so as to be readily separable from water, separating the coated particles from superfluous water, and forming them into briquettes.

55 7. A process for making briquettes from carbonized fuel which consists in suspending suitably divided carbonized fuel in water so as to form a freely flowing pulp, adding to the pulp slaked lime and also a binding

medium, subjecting the pulp to agitation, 65 whereby carbonized particles are coated with binding medium and flocculated so as to be readily separable from water, separating the coated particles from superfluous water, and forming them into briquettes.

70 8. The process of making briquettes of purified material from impure material which consists in treating the impure material in suitably divided condition whereby selected particles are separated from impurities, agitating the selected particles in a freely flowing pulp with a binding medium having an affinity for the selected particles so as to coat such particles with binding 75 medium and agglomerate them, and separating the resulting agglomerates from pulp liquid and forming the same into briquettes.

80 9. A process of making briquettes of carbonized fuel which consists in treating impure carbonized fuel in suitably divided condition so as to separate impurities therefrom, agitating the purified carbonized particles in a freely flowing pulp with a binding medium having an affinity for the carbonized particles so as to coat carbonized particles with 85 binding medium and agglomerate them, and separating the resulting agglomerates from pulp liquid and forming the same into briquettes.

90 10. A process of obtaining relatively dry agglomerates of purified carbonized fuel which consists in treating the impure carbonized fuel in suitably divided condition so as to separate impurities therefrom, agitating the purified carbonized particles in a 95 freely flowing pulp with a fluid having an affinity for the carbonized particles so as to coat carbonized particles with the fluid and agglomerate them, and separating the resulting agglomerates from pulp liquid.

100 11. A process of making fuel briquettes from impure carbonized fuel which consists in subjecting the crude material in a suitably divided condition to concentration by a froth-flotation process, agitating the concentrates in aqueous suspension with a binding medium and with a saline flocculating agent so that the concentrated carbonized particles become coated with the binding medium and flocculated, separating the resulting coated 105 particles from superfluous water, and forming them into briquettes.

115 12. A process of making fuel briquettes from impure carbonized fuel which consists in subjecting the crude material in a suitably divided condition to concentration by a froth-flotation process, agitating the concentrates in aqueous suspension with a liquified bituminous binding medium and with a saline flocculating agent so that the concentrated carbonized particles become coated with the binding medium and flocculated, separating the coated particles from super- 120 125

fluous water, and forming them into briquettes.

13. A process of making briquettes of carbonized fuel which consists in treating the impure carbonized fuel in suitably divided condition so as to separate impurities therefrom, agitating the purified carbonized particles in a freely flowing pulp with material acting as frothing agent and binding medium so as to coat carbonized particles and agglomerate them and float agglomerates of carbonized particles, and separating the floating agglomerates from pulp liquid and forming the agglomerates into briquettes.

14. A process of making relatively dry agglomerates of purified carbonized fuel which consists in treating the impure carbonized fuel in suitably divided condition so as to separate impurities therefrom, agitating the purified carbonized particles in a freely flowing pulp with material acting as frothing agent and binding medium so as to coat carbonized particles and agglomerate them and float agglomerates of carbonized particles, and separating the floating agglomerates from pulp liquid.

15. A process of making briquettes of purified material from impure material which consists in subjecting the impure material in a suitably divided condition to froth-flotation separation, whereby selected particles are separated from impurities, agitating the selected particles in aqueous suspension with material acting as frothing agent and binding medium and with a flocculating agent, whereby the selected particles become coated, flocculated, and floated in the form of agglomerates supported by bubbles, collecting and draining the float, and forming briquettes from the coated particles.

16. A process of making fuel briquettes from impure carbonized fuel which consists in subjecting the crude material to concentration by a froth-flotation process, agitating the concentrate in aqueous suspension with material acting as both a frothing agent and a binding medium and with a saline flocculating agent whereby carbonized particles become coated with the binding medium, flocculated, and floated in the form of agglomerates supported by bubbles collecting and draining the float, and forming briquettes from the coated particles.

17. A process of making briquettes of carbonized fuel which consists in treating the impure carbonized fuel in suitably divided condition so as to separate impurities therefrom, agitating the purified carbonized particles in a freely flowing pulp, with material acting as frothing agent and binding medium in amount sufficient to cause carbonized particles to agglomerate but insufficient

to flow on the surface of the particles after 65 coating the same, so as to coat carbonized particles and agglomerate them and float agglomerates of carbonized particles, and separating the floating agglomerates from pulp liquid and forming the agglomerates 70 into briquettes.

18. A process of making relatively dry agglomerates of purified carbonized fuel which consists in treating the impure carbonized fuel in suitably divided condition so 75 as to separate impurities therefrom, agitating the purified carbonized particles in a freely flowing pulp, with material acting as frothing agent and binding medium in amount sufficient to cause carbonized particles to agglomerate but insufficient to flow on the surface of the particles after coating the same, so as to coat carbonized particles and agglomerate them and float agglomerates of carbonized particles, and separating the floating agglomerates from pulp liquid.

19. A process of making briquettes of purified material from impure material which consists in subjecting the impure material in suitably divided condition to concentration by froth flotation, whereby selected particles are separated from impurities, agitating the selected particles in a freely flowing pulp with a binding medium having an affinity for the selected particles so as to coat such particles with binding medium and agglomerate them, and separating the resulting agglomerates from pulp liquid and forming the same into briquettes.

20. A process of making briquettes of carbonized fuel which consists in agitating the carbonized fuel in suitably divided condition in a freely flowing pulp, with a sufficient amount of binding medium having an affinity for the carbonized particles to cause them to agglomerate but insufficient binding medium to flow on the surface of the particles after it has coated the same, so as to coat carbonized particles with binding medium and agglomerate them, and separating the resulting agglomerates from pulp liquid and forming the same into briquettes.

21. A process of making briquettes of carbonized fuel which consists in treating impure carbonized fuel in suitably divided condition so as to separate impurities therefrom, agitating the purified carbonized particles in a freely flowing pulp, with a sufficient amount of binding medium having an affinity for the carbonized particles to cause them to agglomerate but insufficient binding medium to flow on the surface of the particles after it has coated the same, so as to coat carbonized particles with binding medium and agglomerate them, and separating the resulting agglomerates from pulp liquid and forming the same into briquettes.

22. A process of making relatively dry agglomerates of purified carbonized fuel which consists in treating the impure carbonized fuel in suitably divided condition so as to separate impurities therefrom, agitating the purified carbonized particles in a freely flowing pulp, with a sufficient amount of a fluid having an affinity for the carbonized particles to cause them to agglomerate but insufficient of the fluid to flow on the surface of the particles after it has coated the same, so as to coat carbonized particles with the fluid and agglomerate them, and separating the resulting agglomerates from pulp liquid. 65
23. A process of making briquettes of carbonized fuel which consists in subjecting the crude material in suitably divided condition to concentration by froth flotation, agitating the concentrates in a freely flowing pulp with a binding medium having an affinity for the carbonized particles so as to coat carbonized particles with binding medium and agglomerate them, and separating the resulting agglomerates from pulp liquid and forming the same into briquettes. 70
24. A process of forming relatively dry agglomerates of purified carbonized fuel which consists in subjecting the crude material in suitably divided condition to concentration by froth flotation, agitating the concentrates in a freely flowing pulp with a fluid having an affinity for the carbonized particles so as to coat carbonized particles with the fluid and agglomerate them, and separating the resulting agglomerates from pulp liquid. 75
25. A process of making briquettes of carbonized fuel which consists in subjecting the crude material in suitably divided condition to concentration by froth flotation, agitating the concentrates in a freely flowing pulp with a sufficient amount of binding medium having an affinity for the carbonized particles to cause them to agglomerate but insufficient binding medium to flow on the surface of the particles after it has coated the same, so as to coat carbonized particles with binding medium and agglomerate them, and separating the resulting agglomerates from pulp liquid and forming the same into briquettes. 80
26. A process of making relatively dry agglomerates of purified carbonized fuel which consists in subjecting the crude material in suitably divided condition to concentration by froth flotation, agitating the concentrates in a freely flowing pulp, with a sufficient amount of a fluid having an affinity for the carbonized particles to cause them to agglomerate but insufficient of the fluid to flow on the surface of the particles after it has coated the same, so as to coat carbonized particles with the fluid and agglomerate them and separating the resulting agglomerates from pulp liquid. 85
27. A process of making briquettes of carbonized fuel which consists in subjecting the crude material in suitably divided condition to concentration by froth flotation, agitating the concentrates in a freely flowing pulp, with material acting as frothing agent and binding medium so as to coat carbonized particles and agglomerate them and float agglomerates of the particles, and separating the floating agglomerates from pulp liquid and forming the agglomerates into briquettes. 90
28. A process of making relatively dry agglomerates of purified carbonized fuel which consists in subjecting the crude material in suitably divided condition to concentration by froth flotation, agitating the purified carbonized particles in a freely flowing pulp with material acting as frothing agent and binding medium so as to coat carbonized particles and agglomerate them and float agglomerates of the particles, and separating the floating agglomerates from pulp liquid and forming the agglomerates into briquettes. 95
29. A process of making briquettes of carbonized fuel which consists in subjecting the crude material in suitably divided condition to concentration by froth flotation, agitating the concentrates in a freely flowing pulp, with material acting as frothing agent and binding medium in amount sufficient to cause carbonized particles to agglomerate but insufficient to flow on the surface of the particles after coating the same, so as to coat carbonized particles and agglomerate them and float agglomerates of the particles, and separating the floating agglomerates from pulp liquid and forming the agglomerates into briquettes. 100
30. A process of making relatively dry agglomerates of purified carbonized fuel which consists in subjecting the crude material in suitably divided condition to concentration by froth flotation, agitating the concentrates in a freely flowing pulp, with material acting as frothing agent and binding medium in amount sufficient to cause carbonized particles to agglomerate but insufficient to flow on the surface of the particles after coating the same, so as to coat carbonized particles and agglomerate them and float agglomerates of carbonized particles, and separating the floating agglomerates from pulp liquid. 105
31. A process of making briquettes which consists in suspending suitably divided solids in water so as to form a freely flowing pulp and subjecting the pulp to agitation with a binding medium containing a large proportion of heavy hydrocarbons so as to coat solid particles with binding medium and agglomerate them and separating the resulting agglomerates from pulp liquid. 110
32. A process of making briquettes which consists in suspending suitably divided solids in water so as to form a freely flowing pulp and subjecting the pulp to agitation with a binding medium containing a large proportion of heavy hydrocarbons so as to coat solid particles with binding medium and agglomerate them and separating the resulting agglomerates from pulp liquid. 115
33. A process of making briquettes which consists in suspending suitably divided solids in water so as to form a freely flowing pulp and subjecting the pulp to agitation with a binding medium containing a large proportion of heavy hydrocarbons so as to coat solid particles with binding medium and agglomerate them and separating the resulting agglomerates from pulp liquid. 120
34. A process of making briquettes which consists in suspending suitably divided solids in water so as to form a freely flowing pulp and subjecting the pulp to agitation with a binding medium containing a large proportion of heavy hydrocarbons so as to coat solid particles with binding medium and agglomerate them and separating the resulting agglomerates from pulp liquid. 125

glomerate them, and separating the resulting agglomerates from pulp liquid and forming the same into briquettes.

32. A process of making briquettes of carbonized fuel which consists in agitating the carbonized fuel in suitably divided condition in a freely flowing pulp with a binding medium containing a large proportion of heavy hydrocarbons so as to coat the particles with binding medium and agglomerate the particles, and separating the resulting agglomerates from pulp liquid and forming the same into briquettes.

33. A process of making briquettes of carbonized fuel which consists in treating impure carbonized fuel in suitably divided condition so as to separate impurities therefrom, agitating the purified carbonized particles in a freely flowing pulp with a binding medium containing a large proportion of heavy hydrocarbons so as to coat carbonized particles with binding medium and agglomerate them, and separating the resulting agglomerates from pulp liquid and forming the same into briquettes.

34. A process of making relatively dry agglomerates of purified carbonized fuel which consists in treating the impure carbonized fuel in suitably divided condition so as to separate impurities therefrom, agitating the purified carbonized particles in a freely flowing pulp with a fluid containing a large proportion of heavy hydrocarbons so as to coat carbonized particles with the fluid and agglomerate them, and separating the resulting agglomerates from pulp liquid.

35. A process of making briquettes of carbonized fuel which consists in treating the impure carbonized fuel in suitably divided condition so as to separate impurities therefrom, agitating the purified carbonized particles in a freely flowing pulp with material acting as frothing agent and binding medium and containing a large proportion of heavy hydrocarbons so as to coat carbonized particles and agglomerate them and float agglomerates of the particles, and separating the floating agglomerates from pulp liquid and forming the agglomerates into briquettes.

36. A process of making relatively dry agglomerates of purified carbonized fuel which consists in treating the impure carbonized fuel in suitably divided condition so as to separate impurities therefrom, agitating the purified carbonized particles in a freely flowing pulp, with material acting as frothing agent and binding medium and containing a large proportion of heavy hydrocarbons, so as to coat carbonized particles and agglomerate them and float agglomerates of the particles, and separating the floating agglomerates from pulp liquid.

37. A process of making briquettes of car-

bonized fuel which consists in treating the impure carbonized fuel in suitably divided condition so as to separate impurities therefrom, agitating the purified carbonized particles in a freely flowing pulp, with a sufficient amount of material acting as frothing agent and binding medium and containing a large proportion of heavy hydrocarbons to cause carbonized particles to agglomerate but insufficient to flow on the surface of the particles after coating the same, so as to coat carbonized particles and agglomerate them and float agglomerates of the particles, and separating the floating agglomerates from pulp liquid and forming the agglomerates into briquettes.

38. A process of making relatively dry agglomerates of purified carbonized fuel which consists in treating the impure carbonized fuel in suitably divided condition so as to separate impurities therefrom, agitating the purified carbonized particles in a freely flowing pulp, with a sufficient amount of material acting as frothing agent and binding medium and containing a large proportion of heavy hydrocarbons to cause carbonized particles to agglomerate but insufficient to flow on the surface of the particles after coating the same, so as to coat carbonized particles and agglomerate them and float agglomerates of carbonized particles, and separating the floating agglomerates from pulp liquid.

39. A process of making briquettes of purified material from impure material which consists in subjecting the impure material in suitably divided condition to concentration by froth flotation, whereby selected particles are separated from impurities, agitating the selected particles in a freely flowing pulp with a binding medium containing a large proportion of heavy hydrocarbons so as to coat such particles with binding medium and agglomerate them, and separating the resulting agglomerates from pulp liquid and forming the same into briquettes.

40. A process of making briquettes of carbonized fuel which consists in agitating the carbonized fuel in suitably divided condition in a freely flowing pulp, with a sufficient amount of a binding medium containing a large proportion of heavy hydrocarbons to cause carbonized particles to agglomerate but insufficient binding medium to flow on the surface of the particles after it has coated the same, so as to coat carbonized particles with binding medium and agglomerate them, and separating the resulting agglomerates from pulp liquid and forming the same into briquettes.

41. A process of making briquettes of carbonized fuel which consists in treating impure carbonized fuel in suitably divided

- condition so as to separate impurities therefrom, agitating the purified carbonized particles in a freely flowing pulp, with a sufficient amount of a binding medium containing a large proportion of heavy hydrocarbons to cause carbonized particles to agglomerate but insufficient binding medium to flow on the surface of the particles after it has coated the same, so as to coat carbonized particles with binding medium and agglomerate them, and separating the resulting agglomerates from pulp liquid and forming the same into briquettes.
42. A process of making relatively dry agglomerates of purified carbonized fuel which consists in treating the impure carbonized fuel in suitably divided condition so as to separate impurities therefrom, agitating the purified carbonized particles in a freely flowing pulp, with a sufficient amount of a fluid containing a large proportion of heavy hydrocarbons to cause carbonized particles to agglomerate but insufficient of the fluid to flow on the surface of the particles after it has coated the same, so as to coat carbonized particles with the fluid and agglomerate them, and separating the resulting agglomerates from pulp liquid.
43. A process of making briquettes of carbonized fuel which consists in subjecting the crude material in suitably divided condition to concentration by froth flotation, agitating the concentrates in a freely flowing pulp with a binding medium containing a large proportion of heavy hydrocarbons so as to coat carbonized particles with binding medium and agglomerate them, and separating the resulting agglomerates from pulp liquid and forming the same into briquettes.
44. A process of making relatively dry agglomerates of purified carbonized fuel which consists in subjecting the crude material in suitably divided condition to concentration by froth flotation, agitating the concentrates in a freely flowing pulp with a fluid containing a large proportion of heavy hydrocarbons so as to coat carbonized particles with the fluid and agglomerate them, and separating the resulting agglomerates from pulp liquid.
45. A process of making briquettes of carbonized fuel which consists in subjecting the crude material in suitably divided condition to concentration by froth flotation, agitating the concentrates in a freely flowing pulp, with a sufficient amount of binding medium containing a large proportion of heavy hydrocarbons to cause carbonized particles to agglomerate but insufficient binding medium to flow on the surface of the particles after it has coated the same so as to coat carbonized particles with binding medium and agglomerate them, and separating the resulting agglomerates from pulp liquid and forming the same into briquettes.
46. A process of making relatively dry agglomerates of purified carbonized fuel which consists in subjecting the crude material in suitably divided condition to concentration by froth flotation, agitating the concentrates in a freely flowing pulp, with a sufficient amount of a fluid containing a large proportion of heavy hydrocarbons to cause carbonized particles to agglomerate but insufficient of the fluid to flow on the surface of the particles after it has coated the same, so as to coat carbonized particles with the fluid and agglomerate them, and separating the resulting agglomerates from pulp liquid.
47. A process of making briquettes of carbonized fuel which consists in subjecting the crude material in suitably divided condition to concentration by froth flotation, agitating the concentrates in a freely flowing pulp, with material acting as frothing agent and binding medium and containing a large proportion of heavy hydrocarbons so as to coat carbonized particles and agglomerate them and float agglomerates of the particles, and separating the floating agglomerates from pulp liquid and forming the agglomerates into briquettes.
48. A process of making relatively dry agglomerates of purified carbonized fuel which consists in subjecting the crude material in suitably divided condition to concentration by froth flotation, agitating the purified carbonized particles in a freely flowing pulp with material acting as frothing agent and binding medium and containing a large proportion of heavy hydrocarbons so as to coat carbonized particles and agglomerate them and float agglomerates of the particles, and separating the floating agglomerates from pulp liquid and forming the agglomerates into briquettes.
49. A process of making briquettes of carbonized fuel which consists in subjecting the crude material in suitably divided condition to concentration by froth flotation, agitating the concentrates in a freely flowing pulp, with a sufficient amount of material acting as frothing agent and binding medium and containing a large proportion of heavy hydrocarbons to cause carbonized particles to agglomerate but insufficient to flow on the surface of the particles after coating the same so as to coat carbonized particles and agglomerate them and float agglomerates of the particles, and separating the floating agglomerates from pulp liquid and forming the agglomerates into briquettes.
50. A process of making relatively dry agglomerates of purified carbonized fuel which consists in subjecting the crude material in suitably divided condition to concentration by froth flotation, agitating the concentrates in a freely flowing pulp, with a sufficient amount of material acting as

- frothing agent and binding medium and containing a large proportion of heavy hydrocarbons to cause carbonized particles to agglomerate but insufficient to flow on the surface of the particles after coating the same, so as to float agglomerates of the particles, and separating the floating agglomerates from pulp liquid.
51. A process of making briquettes which consists in suspending suitably divided solids in water so as to form a freely flowing pulp and subjecting the pulp to agitation with pitch so as to coat solid particles with pitch and agglomerate them, and separating the resulting agglomerates from pulp liquid and forming the same into briquettes.
52. A process of making briquettes of carbonized fuel which consists in agitating the carbonized fuel in suitably divided condition in a freely flowing pulp with pitch so as to coat carbonized particles with pitch and agglomerate them, and separating the resulting agglomerates from pulp liquid and forming the same into briquettes.
53. A process of making briquettes which consists in agitating suitably divided solids in a freely flowing pulp with a flocculating agent and pitch so as to coat solid particles with pitch and agglomerate them, and separating the resulting agglomerates from pulp liquid and forming the same into briquettes.
54. A process of making briquettes of purified material from impure material which consists in subjecting the impure material in suitably divided condition to concentration by froth flotation, whereby selected particles are separated from impurities, agitating the selected particles in a freely flowing pulp with pitch so as to coat such particles with pitch and agglomerate them and separating the resulting agglomerates from pulp liquid and forming the same into briquettes.
55. A process of making briquettes of carbonized fuel which consists in subjecting the crude material in suitably divided condition to concentration by froth flotation, agitating the concentrates in a freely flowing pulp with pitch so as to coat carbonized particles with pitch and agglomerate them, and separating the resulting agglomerates from pulp liquid and forming the same into briquettes.
56. A process of making briquettes of carbonized fuel which consists in subjecting the crude material in suitably divided condition to concentration by froth flotation, agitating the concentrates in a freely flowing pulp, with a sufficient amount of pitch to cause carbonized particles to agglomerate but insufficient pitch to flow on the surface of the particles after it has coated the same, so as to coat carbonized particles with pitch and agglomerate them, and separating the resulting agglomerates from pulp liquid and forming the same into briquettes.
57. A process of making briquettes of carbonized fuel which consists in subjecting the crude material in suitably divided condition to concentration by froth flotation, agitating the concentrates in a freely flowing pulp with material affording a frothing agent and containing pitch so as to coat carbonized particles and agglomerate them and float agglomerates of the particles, and separating the floating agglomerates from pulp liquid and forming the agglomerates into briquettes.
58. A process of making briquettes of carbonized fuel which consists in subjecting the crude material in suitably divided condition to concentration by froth flotation, agitating the concentrates in a freely flowing pulp, with a sufficient amount of material affording a frothing agent and containing pitch to cause carbonized particles to agglomerate but insufficient to flow on the surface of the particles after coating the same, so as to coat carbonized particles and agglomerate them and float agglomerates of the particles, and separating the floating agglomerates from pulp liquid and forming the agglomerates into briquettes.
59. A process of making briquettes which consists in suspending suitably divided solids in water so as to form a freely flowing pulp and subjecting the pulp to agitation with a binding medium having an affinity for solid particles in amount sufficient to cause particles to agglomerate but insufficient to flow on the surface of the particles after coating the same, so as to coat solid particles with binding medium and agglomerate them, and separating the resulting agglomerates from pulp liquid and forming the same into briquettes.
60. A process of making briquettes of purified material from impure material which consists in treating the impure material in suitably divided condition whereby selected particles are separated from impurities, agitating the selected particles in a freely flowing pulp with a binding medium having an affinity for solid particles in amount sufficient to cause particles to agglomerate but insufficient to flow on the surface of the particles after coating the same, so as to coat such particles with binding medium and agglomerate them, and separating the resulting agglomerates from pulp liquid and forming the same into briquettes.
61. A process of making briquettes of purified material from impure material which consists in subjecting the impure material in suitably divided condition to concentration by froth flotation, whereby selected particles are separated from impurities,

agitating the selected particles in a freely flowing pulp with a binding medium having an affinity for the selected particles in amount sufficient to cause the particles to agglomerate but insufficient to flow on the surface of the particles after coating the same, so as to coat such particles with a binding medium and agglomerate them, and separating the resulting agglomerates from pulp liquid and forming the same into briquettes.

In testimony whereof we have signed our names to this specification in the presence of two subscribing witnesses.

WALTER BROADBRIDGE.

EDWIN EDSER.

WILLIAM WARWICK STENNING.

Witnesses:

HOWARD CHARLES HAWKINS,

KENNETH L. STEWARD.